

# United States Patent [19]

Kakimi

[11] Patent Number: 4,871,641

[45] Date of Patent: \* Oct. 3, 1989

[54] **LIGHT-SENSITIVE MATERIAL  
CONTAINING SILVER HALIDE REDUCING  
AGENT AND POLYMERIZABLE  
COMPOUND AND PROCESS FOR  
PREPARATION THEREOF**

[75] Inventor: Fujio Kakimi, Minami-ashigara,  
Japan

[73] Assignee: Fuji Photo Film Co., Ltd., Kanagawa,  
Japan

[\*] Notice: The portion of the term of this patent  
subsequent to Apr. 5, 2005 has been  
disclaimed.

[21] Appl. No.: 24,431

[22] Filed: Mar. 11, 1987

## [30] Foreign Application Priority Data

Mar. 11, 1986 [JP] Japan 61-52994

[51] Int. Cl.<sup>4</sup> G03C 1/42; G03C 11/68

[52] U.S. Cl. 430/138; 430/264;  
430/281

[58] Field of Search 430/138, 270, 281, 264

## [56] References Cited

### U.S. PATENT DOCUMENTS

4,501,809 2/1985 Hiraishi et al. .... 430/138  
4,529,681 7/1985 Usami et al. .... 430/138  
4,629,676 12/1986 Hayakawa et al. .... 430/330  
4,735,884 4/1988 Tsukahara et al. .... 430/138

### FOREIGN PATENT DOCUMENTS

0203613 12/1986 European Pat. Off. .... 430/203

Primary Examiner—Richard L. Schilling  
Attorney, Agent, or Firm—Sughrue, Mion, Zinn,  
Macpeak & Seas

## [57] ABSTRACT

A light-sensitive material comprising a light-sensitive layer which contains silver halide, a reducing agent and a polymerizable compound provided on a support, characterized in that the silver halide and the polymerizable compound are together contained in microcapsules which are dispersed in the light-sensitive layer, and the light-sensitive layer further contains a binder which is arranged outside of the microcapsules. A process for the preparation thereof is also disclosed.

13 Claims, No Drawings

**LIGHT-SENSITIVE MATERIAL CONTAINING  
SILVER HALIDE REDUCING AGENT AND  
POLYMERIZABLE COMPOUND AND PROCESS  
FOR PREPARATION THEREOF**

**BACKGROUND OF THE INVENTION**

**1. Field of the Invention**

This invention relates to a light-sensitive material comprising a light-sensitive layer containing silver halide, a reducing agent and a polymerizable compound provided on a support and process for the preparation thereof.

**2. Description of Prior Arts**

Light-sensitive materials comprising a light-sensitive layer containing silver halide, a reducing agent and a polymerizable compound provided on a support can be used in an image forming method in which a latent image of silver halide is formed, and then the polymerizable compound is polymerized to form the corresponding image.

Examples of said image forming methods are described in Japanese Patent Publication Nos. 45(1970)-11149 (corresponding to U.S. Pat. No. 3,697,275), 47(1972)-20741 (corresponding to U.S. Pat. No. 3,687,667) and 49(1974)-10697, and Japanese Patent Provisional Publication Nos. 57(1982)-138632, 57(1982)-142638, 57(1982)-176033, 57(1982)-211146 (corresponding to U.S. Pat. No. 4,557,997), 58(1983)-107529 (corresponding to U.S. Pat. No. 4,560,637), 58(1983)-121031 (corresponding to U.S. Pat. No. 4,547,450) and 58(1983)-169143. In these image forming methods, when the exposed silver halide is developed using a developing solution, the polymerizable compound is induced to polymerize in the presence of a reducing agent (which is oxidized) to form a polymer image. Thus, these methods need a wet development process employing a developing solution. Therefore, the process takes a relatively long time.

An improved image forming method employing a dry process is described in Japanese Patent Provisional Publication Nos. 61(1986)-69062 and 61(1986)-73145 (the contents of both publications are described in U.S. Pat. No. 4,629,676 and European Patent Provisional Publication No. 0174634A2). In this image forming method, a recording material (i.e., light-sensitive material) comprising a light-sensitive layer containing a light-sensitive silver salt (i.e., silver halide), a reducing agent, a cross-linkable compound (i.e., polymerizable compound) and a binder provided on a support is imagewise exposed to form a latent image, and then the material is heated to polymerize within the area where the latent image of the silver halide has been formed. The above method employing the dry process and the light-sensitive material employable for such method are also described in Japanese Patent Provisional Publication Nos. 61(1986)-183640, 61(1986)-188535 and 61(1986)-228441.

The above-mentioned image forming methods are based on the principle in which the polymerizable compound is polymerized within the area where a latent image of the silver halide has been formed.

Further, Japanese Patent Provisional Publication No. 61(1986)-260241 (corresponding to U.S. Patent Ser. No. 854,640) describes another image forming method in which the polymerizable compound within the area where a latent image of the silver halide has not been formed is polymerized. In this method, when the mate-

rial is heated, the reducing agent functions as polymerization inhibitor in the portion where a latent image of the silver halide has been formed, and the polymerizable compound within the other area is polymerized.

5 In the light-sensitive material employed in the image forming method, the silver halide and the polymerizable compound can be contained in a microcapsule. The light-sensitive material containing such microcapsules has an advantage in that the reaction to accelerate (or, to inhibit) the polymerization within the area where a latent image of silver halide has been formed can smoothly progress. In handling the light-sensitive material employing the microcapsules, care should be taken to avoid destruction of the microcapsules in the preparation, the preservation, the transference or the image formation thereof.

**SUMMARY OF THE INVENTION**

An object of the present invention is to provide a light-sensitive material which is easy to handle.

Another object of the invention is to provide a light-sensitive material which gives a clear image.

There is provided by the present invention a light-sensitive material comprising a light-sensitive layer which contains silver halide, a reducing agent and a polymerizable compound provided on a support, characterized in that the silver halide and the polymerizable compound are together contained in microcapsules which are dispersed in the light-sensitive layer, and the light-sensitive layer further contains a binder which is arranged outside of the microcapsules.

The above-described light-sensitive material can be advantageously prepared by a process which comprises:

35 adding a binder to a microcapsule dispersion containing silver halide, a reducing agent and a polymerizable compound to obtain a coating solution, wherein the silver halide and the polymerizable compound are together contained in the microcapsules, and

coating the coating solution on the support.

The light-sensitive material of the invention is characterized in that the light-sensitive layer contains a binder which is arranged outside of the microcapsules.

In the light-sensitive material of the invention, the microcapsules in the light-sensitive layer are protected and fixed on the support by the binder. Therefore, the light-sensitive material of the invention is easy to handle in the preparation, the preservation, the transference or the image formation thereof.

50 In the preparation of the light-sensitive material, a microcapsule dispersion is preferably used as a coating solution of the light-sensitive layer. It is difficult, however, to uniformly disperse the microcapsules in the coating solution without destroying the microcapsules. The present inventor has found that the binder has a function of dispersing the microcapsules in the coating solution as well as keeping thus dispersed state in the light-sensitive layer. Therefore, the light-sensitive material of the invention can give an improved clear uniform image, because the microcapsules are kept in the uniformly dispersed state.

**DETAILED DESCRIPTION OF THE  
INVENTION**

In the light-sensitive material of the invention, there is no specific limitation with respect to the binder, and various binders including the known compounds in the

conventional photographic technology can be used. The binder generally is a high molecular compound having a molecular weight of from 1,000 to 10,000,000. The molecular weight more preferably is from 10,000 to 5,000,000.

Examples of the binders preferably employable for the light-sensitive material of the invention include water-insoluble synthetic high molecular compounds, such as styrene/butadiene rubber, styrene/butadiene/acrylonitrile copolymer, styrene/butadiene/maleic anhydride copolymer, acrylate and vinyl acetate; water-soluble natural high molecular compounds, such as protein (e.g., gelatin, albumin, casein), cellulose (including cellulose derivatives, such as carboxymethyl cellulose and hydroxyethyl cellulose), agar-agar, starch (including carboxymethyl starch and starch phosphate), sodium alginate; and water-soluble synthetic high molecular compounds, such as polyvinyl alcohol, polyvinyl pyrrolidone, polyacrylic acid, polyacrylamide, isobutylene/maleic anhydride copolymer, polyvinyl benzenesulfonic acid and the salts of these compounds.

In the light-sensitive layer, the binder is preferably in a state of fixing the microcapsules on the support. More preferably, the binder essentially covers the whole surface of the microcapsules.

In the case that heat development is utilized in the use of the light-sensitive material, the binder preferably is a compound having a low transmission coefficient for oxygen to eliminate the influence of oxygen in the air in the heat development, because oxygen is observed to function as a polymerization inhibitor. The transmission coefficient of oxygen preferably is not more than  $1.0 \times 10^{-11} \text{ cm}^3 \cdot \text{cm} / \text{cm}^2 \cdot \text{sec} \cdot \text{cmHg}$ . The transmission coefficient of oxygen follows the definition described in J. Brandrup, edited by E. H. Immergut, "Polymer Handbook", (1975, III-229). The above value of the transmission coefficient of oxygen substantially corresponds to not more than about  $5 \times 10^{-10} \text{ cm}^2 / \text{sec}$  determined according to the definition described in K. Petrank, Journal of Applied Polymer Science, Vol. 23, 2365 (1979).

Examples of the above polymer include polyacrylonitrile, acrylonitrile/styrene copolymer, polymethylacrylonitrile, methacrylonitrile/styrene copolymer, polyvinyl acetate, polyvinyl alcohol, polyvinyl chloride, polyvinylidene chloride, polyvinyl imidazole, vinylidene chloride/acrylonitrile copolymer, polyacrylamide, vinyl alcohol/ethylene copolymer (tradename "Eval" produced by Kuraray Co., Ltd.) and gelatin.

These polymers are described in the above Polymer Handbook and Journal of Applied Polymer Science.

The binder can be used singly or in combination with two or more compounds.

The binder is preferably used in an amount ranging from 10 to 50 weight %, based on the amount of the microcapsules.

The microcapsule containing the silver halide and the polymerizable compound, the reducing agent, and the support which constitute the light-sensitive material of the invention with the binder are described below. Thus composed material is referred to hereinafter as "light-sensitive material".

There is no specific limitation with respect to the silver halide contained in the light-sensitive layer of the light-sensitive material.

Examples of the silver halides include silver chloride, silver bromide, silver iodide, silver chlorobromide, sil-

ver chloroiodide, silver iodobromide, and silver chloroiodobromide in the form of grains.

The halogen composition of individual grains may be homogeneous or heterogeneous. The heterogeneous grains having a multilayered structure in which the halogen composition varies from the core to the outer shell (see Japanese Patent Provisional Publication Nos. 57(1982)-154232, 58(1983)-108533, 59(1984)-48755 and 59(1984)-52237, U.S. Pat. No. 4,433,048, and European Pat. No. 100,984) can be employed.

There is no specific limitation on the crystal habit of silver halide grains. Two or more kinds of silver halide grains which differ in halogen composition, crystal habit, grain size, and/or other features from each other can be used in combination. There is no specific limitation on grain size distribution of silver halide grains. The silver halide grains ordinarily have a mean size of 0.001 to 5  $\mu\text{m}$ , more preferably 0.001 to 2  $\mu\text{m}$ .

The total silver content (including silver halide and an organic silver salt which is one of optional components) in the light-sensitive layer preferably is in the range of from 0.1  $\text{mg}/\text{m}^2$  to 10  $\text{g}/\text{m}^2$ . The silver content of the silver halide in the light-sensitive layer preferably is not more than 1  $\text{g}/\text{m}^2$ , more preferably in the range of from 1  $\text{mg}$  to 500  $\text{mg}/\text{m}^2$ .

The reducing agent employed in the light-sensitive material has a function of reducing the silver halide and/or a function of accelerating or restraining polymerization of the polymerizable compound. Examples of the reducing agents having these functions include various compounds, such as hydroquinones, catechols, p-aminophenols, p-phenylenediamines, 3-pyrazolidones, 3-aminopyrazoles, 4-amino-5-pyrazolones, 5-aminouracils, 4,5-dihydroxy-6-aminopyrimidines, reductones, aminoreductones, o- or p-sulfonamido-phenols, o- or p-sulfonamidonaphthols, 2-sulfonamidoindanones, 4-sulfonamido-5-pyrazolones, 3-sulfonamidoindoless, sulfonamidopyrazolotriazoles,  $\alpha$ -sulfonamidoketones, hydrazines, etc. Depending on the nature or amount of the reducing agent, the polymerizable compound within either an area where a latent image of the silver halide has been formed or an area where a latent image of the silver halide has not been formed can be polymerized. In the developing system in which the polymerizable compound within the area where the latent image has not been formed is polymerized, 1-phenyl-3-pyrazolidone is preferably employed as the reducing agent.

The light-sensitive materials employing the reducing agent having these functions (including compounds referred to as developing agent or hydrazine derivative) are described in Japanese Patent Provisional Publication Nos. 61(1986)-183640, 61(1986)-188535 and 61(1986)-228441, and Japanese Patent Application Nos. 60(1985)-210657, 60(1985)-226084, 60(1985)-227527 and 60(1985)-227528. These reducing agents are also described in T. James, "The Theory of the Photographic Process", 4th edition, 291-334 (1977), Research Disclosure No. 17029, 9-15 (June 1978), and Research Disclosure No. 17643, 22-31 (December 1978). The reducing agents described in these publications and applications can be employed in the light-sensitive material of the present invention. Thus, "the reducing agent(s)" in the present specification means to include all of the reducing agents described in the above mentioned publications and applications.

These reducing agents can be used singly or in combination. In the case that two or more reducing agents are used in combination, certain interactions between these reducing agents may be expected. One of the interactions is for acceleration of reduction of silver halide (and/or an organic silver salt) through so-called superadditivity. Another interaction is a chain reaction in which an oxidized state of one reducing agent formed by a reduction of silver halide (and/or an organic silver salt) induces or inhibits the polymerization of the polymerizable compound via oxidation-reduction reaction with another reducing agent. Both interactions may occur simultaneously. Thus, it is difficult to determine which of the interactions has occurred in practical use.

Examples of these reducing agents include pentadecylhydroquinone, 5-t-butylcatechol, p-(N,N-dimethylamino)phenol, 1-phenyl-4-methyl-4-hydroxymethyl-3-pyrazolidone, 1-phenyl-4-methyl-4-heptadecylcarbonyloxymethyl-3-pyrazolidone, 2-phenylsulfonylamino-4-hexadecyloxy-5-t-octylphenol, 2-phenylsulfonylamino-4-t-butyl-5-hexadecyloxyphenol, 2-(N-butylcarbamoyl)-4-phenylsulfonylaminonaphthol, 2-(N-methyl-N-octadecylcarbamoyl)-4-sulfonylaminonaphthol, 1-acetyl-2-phenylhydrazine, 1-acetyl-2-(p- or o-aminophenyl)hydrazine, 1-formyl-2-(p- or o-aminophenyl)hydrazine, 1-acetyl-2-(p- or o-methoxyphenyl)hydrazine, 1-lauroyl-2-(p- or o-aminophenyl)hydrazine, 1-trityl-2-(2,6-dichloro-4-cyanophenyl)hydrazine, 1-trityl-2-phenylhydrazine, 1-phenyl-2-(2,4,6-trichlorophenyl)hydrazine, 1-[2-(2,5-di-tert-pentylphenoxy)-butyloyl]-2-(p- or o-aminophenyl)hydrazine, 1-[2-(2,5-di-tert-pentylphenoxy)butyloyl]-2-(p- or o-aminophenyl)hydrazine pentadecylfluorocaprylate salt, 3-indazolone, 1-(3,5-dichlorobenzoyl)-2-phenylhydrazine, 1-trityl-2-[(2-N-butyl-N-octylsulfamoyl)-4-methanesulfonyl]phenyl]hydrazine, 1-[4-(2,5-di-tert-pentylphenoxy)butyloyl]-2-(p- or o-methoxyphenyl)hydrazine, 1-(methoxycarbonylbenzohydryl)-2-phenylhydrazine, 1-formyl-2-[4-(2-(2,4-di-tert-pentylphenoxy)-butylamide)phenyl]hydrazine, 1-acetyl-2-[4-(2-(2,4-di-tert-pentylphenoxy)butylamido)phenyl]hydrazine, 1-trityl-2-[(2,6-dichloro-4-(N,N-di-2-ethylhexyl)carbamoyl)phenyl]hydrazine, 1-(methoxycarbonylbenzohydryl)-2-(2,4-dichlorophenyl)hydrazine and 1-trityl-2-[(2-(N-ethyl-N-octylsulfamoyl)-4-methanesulfonyl)phenyl]hydrazine.

The amount of the reducing agent in the light-sensitive layer preferably ranges from 0.1 to 1,500 mole % based on the amount of silver (contained in the silver halide and an organic silver salt).

These reducing agents can be contained in the microcapsule or arranged outside of the microcapsule in the light-sensitive layer. Generally, the reducing agent is preferably contained in the microcapsule, because the reaction can progress smoothly in such case. The reducing agent is more preferably dispersed or dissolved in the core material containing the polymerizable compound. In the case that heat development is utilized in the use of the light-sensitive material, there is no problem in arranging the reducing agent outside of the microcapsule, because the reducing agent can permeate the microcapsule to reach the core material.

There is no specific limitation with respect to the polymerizable compound, and any known polymerizable compounds including monomers, oligomers and polymers can be contained in the light-sensitive layer. In the case that heat development (i.e., thermal development) is utilized for developing the light-sensitive mate-

rial, the polymerizable compounds having a relatively higher boiling point (e.g., 80° C. or higher) that are hardly evaporated upon heating are preferably employed. In the case that the light-sensitive layer contains a color image forming substance, the polymerizable compounds are preferably cross-linkable compounds having plural polymerizable groups in the molecule, because such cross-linkable compounds favorably serve for fixing the color image forming substance in the course of polymerization hardening of the polymerizable compounds.

The polymerizable compound employable for the light-sensitive material of the invention are described in the above-mentioned and later-mentioned publications and applications concerning the light-sensitive material.

Preferred polymerizable compounds employable for the light-sensitive material are compounds which are polymerizable through addition reaction or ring-opening reaction. Preferred examples of the compounds being polymerizable through addition reaction include compounds having an ethylenic unsaturated group. Preferred examples of the compounds being polymerizable through ring-opening reaction include the compounds having an epoxy group. Among them, the compounds having an ethylenic unsaturated group are preferred.

Examples of compounds having an ethylenic unsaturated group include acrylic acid, salts of acrylic acid, acrylic esters, acrylamides, methacrylic acid, salts of methacrylic acid, methacrylic esters, methacrylamide, maleic anhydride, maleic esters, itaconic esters, styrene, styrene derivatives, vinyl ethers, vinyl esters, N-vinyl heterocyclic compounds, allyl ethers, allyl esters, and compounds carrying a group or groups corresponding to one or more of these compounds.

Concrete examples of the acrylic esters include n-butyl acrylate, cyclohexyl acrylate, 2-ethylhexyl acrylate, benzyl acrylate, furfuryl acrylate, ethoxyethoxy acrylate, dicyclohexyloxyethyl acrylate, nonyl-phenoxyethyl acrylate, hexanediol diacrylate, butanediol diacrylate, neopentylglycol diacrylate, trimethylol-propane triacrylate, pentaerythritol tetraacrylate, dipentaerythritol pentaacrylate, diacrylate of polyoxyethylene bisphenol A, polyacrylate of hydroxypolyether, polyester acrylate, and polyurethane acrylate.

Concrete examples of the methacrylic esters include methyl methacrylate, butyl methacrylate, ethylene glycol dimethacrylate, butanediol dimethacrylate, neopentylglycol dimethacrylate, trimethylolpropane trimethacrylate, pentaerythritol trimethacrylate, pentaerythritol tetramethacrylate, and dimethacrylate of polyoxyalkylenated bisphenol A.

The polymerizable compounds can be used singly or in combination of two or more compounds. Further, compounds formed by bonding a polymerizable group such as a vinyl group or a vinylidene group to a reducing agent or a color image forming substance are also employed as the polymerizable compounds. The light-sensitive materials employing these compounds which show functions as both the reducing agent and the polymerizable compound, or of the color image forming substance and the polymerizable compound are included in embodiments of the invention.

The amount of the polymerizable compound for incorporation into the light-sensitive layer preferably ranges from 5 to  $1.2 \times 10^5$  times (by weight) as much as

the amount of silver halide, more preferably from 10 to  $1 \times 10^4$  times as much as the silver halide.

There is no specific limitation on preparation of the microcapsules. There is also no specific limitation with respect to the shell material of the microcapsule, and various known materials such as polymers which are used in the conventional microcapsules can be employed as the shell material. The mean particle size of the microcapsule preferably ranges from 0.5 to 50  $\mu\text{m}$ , more preferably 1 to 25  $\mu\text{m}$ , most preferably 3 to 20  $\mu\text{m}$ .

The light-sensitive material of the invention can be prepared by arranging a light-sensitive layer containing the above-mentioned components on a support. There is no limitation with respect to the support. In the case that heat development is utilized in the use of the light-sensitive material, the material of the support preferably is resistant to heat given in the processing stage. Examples of the material employable for the preparation of the support include glass, paper, fine paper, coat paper, synthetic paper, metals and analogues thereof, polyester, acetyl cellulose, cellulose ester, polyvinyl acetal, polystyrene, polycarbonate, polyethylene terephthalate, and paper laminated with resin or polymer (e.g., polyethylene).

The light-sensitive layer can further contain optional components such as color image forming substances, sensitizing dyes, organic silver salts, various kinds of image formation accelerators, thermal polymerization inhibitors, thermal polymerization initiators, development stopping agents, fluorescent brightening agents, discoloration inhibitors, antihalation dyes or pigments, antiirradiation dyes or pigments, matting agents, antimudging agents, plasticizers and water releasers.

There is no specific limitation with respect to the color image forming substance, and various kinds of substances can be employed. Thus, examples of the color image forming substance include both colored substance (i.e., dyes and pigments) and non-colored or almost non-colored substance (i.e., color former or dye- or pigment-precursor) which develops to give a color under application of external energy (e.g., heating, pressing, light irradiation, etc.) or by contact with other components (i.e., developer). The light-sensitive material using the color image forming substance is described in Japanese Patent Provisional Publication No. 61(1986)-73145.

Examples of the dyes and pigments (i.e., colored substances) employable in the invention include commercially available ones, as well as various known compounds described in the technical publications, e.g., Yuki Gosei Kagaku Kyokai (ed.), Handbook of Dyes (in Japanese, 1970) and Nippon Gomryo Gijutsu Kyokai (ed.), New Handbook of Pigments (in Japanese, 1977). These dyes and pigments can be used in the form of a solution or a dispersion.

Examples of the substances which develop to give a color by certain energy includes thermochromic compounds, piezochromic compounds, photochromic compounds and leuco compounds derived from triarylmethane dyes, quinone dyes, indigoid dyes, azine dyes, etc. These compounds are capable of developing a color by heating, application of pressure, light-irradiation or air-oxidation.

Examples of the substances which develop to give a color in contact with other components include various compounds capable of developing a color through some reaction between two or more components, such as acid-base reaction, oxidation-reduction reaction, cou-

pling reaction, chelating reaction, and the like. Examples of such color formation systems are described in Hiroyuki Moriga, "Introduction of Chemistry of Speciality Paper" (in Japanese, 1975), 29-58 (pressure-sensitive copying paper), 87-95 (azo-graphy), 118-120 (heat-sensitive color formation by a chemical change) or in MSS. of the seminar promoted by the Society of Kinki Chemical Industry, "The Newest Chemistry of Coloring Matter—Attractive Application and New Development as a Functional Coloring Matter", 26-32 (June, 19, 1980). Examples of the color formation systems specifically include a color formation system used in pressure-sensitive papers, etc., comprising a color former having a partial structure of lactone, lactam, spiropyran, etc., and an acidic substance (developer), e.g., acid clay, phenol, etc.; a system utilizing azo-coupling reaction between an aromatic diazonium salt, diazotate or diazosulfonate and naphthol, aniline, active methylene, etc.; a system utilizing a chelating reaction, such as a reaction between hexamethylenetetramine and a ferric ion and gallic acid, or a reaction between a phenolphthalein-complexon and an alkaline earth metal ion; a system utilizing oxidation-reduction reaction, such as a reaction between ferric stearate and pyrogallol, or a reaction between silver behenate and 4-methoxy-1-naphthol, etc.

The color image forming substance in the light-sensitive material is preferably used in an amount of from 0.5 to 50 parts by weight, and more preferably from 2 to 30 parts by weight, per 100 parts by weight of the polymerizable compound. In the case that the developer is used, it is preferably used in an amount of from about 0.3 to about 80 parts by weight per one part by weight of the color former.

There is no specific limitation with respect to the sensitizing dyes, and known sensitizing dyes used in the conventional art of photography may be employed in the light-sensitive material of the invention. Examples of the sensitizing dyes include methine dyes, cyanine dyes, merocyanine dyes, complex cyanine dyes, complex merocyanine dyes, holopolar cyanine dyes, hemicyanine dyes, styryl dyes, and hemioxonol dyes. These sensitizing dyes can be used singly or in combination. Combinations of sensitizing dyes are often used for the purpose of supersensitization. In addition to the sensitizing dyes, a substance which does not per se exhibit spectral sensitization effect or does not substantially absorb visible light but shows supersensitizing activity can be used. The amount of the sensitizing dye to be added generally ranges from about  $10^{-8}$  to about  $10^{-2}$  mol per 1 mol of silver halide. The sensitizing dye is preferably added during the stage of the preparation of the silver halide emulsion.

When the heat development is employed in the use of the light-sensitive material, an organic silver salt is preferably contained in the light-sensitive material. It can be assumed that the organic silver salt takes part in a redox reaction using a silver halide latent image as a catalyst when heated to a temperature of 80° C. or higher. In such case, the silver halide and the organic silver salt preferably are located in contact with each other or close together. Examples of organic compounds employable for forming such organic silver salt include aliphatic or aromatic carboxylic acids, thiocarbonyl group-containing compounds having a mercapto group or an  $\alpha$ -hydrogen atom, imino group-containing compounds, and the like. Among them, benzotriazoles are most preferable. The organic silver salt is preferably

used in an amount of from 0.01 to 10 mol., and preferably from 0.01 to 1 mol., per 1 mol. of the light-sensitive silver halide. Instead of the organic silver salt, an organic compound (e.g., benzotriazole) which can form an organic silver salt in combination with an inorganic silver salt can be added to the light-sensitive layer to obtain the same effect.

Various image formation accelerators are employable in the light-sensitive material. The image formation accelerators have a function to accelerate the oxidation-reduction reaction between a silver halide (and/or an organic silver salt) and a reducing agent, a function to accelerate emigration of an image forming substance from a light-sensitive layer to an image-receiving material or an image-receiving layer, or a similar function. The image formation accelerators can be classified into inorganic bases, organic bases, base precursors, oils, surface active agents, hot-melt solvents, and the like. These groups, however, generally have certain combined functions, i.e., two or more of the above-mentioned effects. Thus, the above classification is for the sake of convenience, and one compound often has a plurality of functions combined.

Various examples of these image formation accelerators are shown below.

Preferred examples of the inorganic bases include hydroxides of alkali metals or alkaline earth metals; secondary or tertiary phosphates, borates, carbonates, quinolinate and metaborates of alkali metals or alkaline earth metals; a combination of zinc hydroxide or zinc oxide and a chelating agent (e.g., sodium picolinate); ammonium hydroxide; hydroxides of quaternary alkylammoniums; and hydroxides of other metals. Preferred examples of the organic bases include aliphatic amines (e.g., trialkylamines, hydroxylamines and aliphatic polyamines); aromatic amines (e.g., N-alkyl-substituted aromatic amines, N-hydroxylalkyl-substituted aromatic amines and bis[p-(dialkylamino)phenyl]methanes), heterocyclic amines, amidines, cyclic amidines, guanidines, and cyclic guanidines. Of these bases, those having a  $pK_a$  of 7 or more are preferred.

The base precursors preferably are those capable of releasing bases upon reaction by heating, such as salts between bases and organic acids capable of decarboxylation by heating, compounds capable of releasing amines through intramolecular nucleophilic substitution, Lossen rearrangement, or Beckmann rearrangement, and the like; and those capable of releasing bases by electrolysis. Preferred examples of the base precursors include guanidine trichloroacetate, piperidine trichloroacetate, morpholine trichloroacetate, p-toluidine trichloroacetate, 2-picoline trichloroacetate, guanidine phenylsulfonylacetate, guanidine 4-chlorophenylsulfonylacetate, guanidine 4-methyl-sulfonylphenylsulfonylacetate, and 4-acetylaminomethyl propionate.

These bases or base precursors are preferably used in an amount of not more than 100% by weight, and more preferably from 0.1 to 40% by weight, based on the total solid content of the light-sensitive layer. These bases or base precursors can be used singly or in combination.

Examples of the oils employable in the invention include high-boiling organic solvents which are used as solvents in emulsifying and dispersing hydrophobic compounds.

Examples of the surface active agents employable in the invention include pyridinium salts, ammonium salts and phosphonium salts as described in Japanese Patent

Provisional Publication No. 59(1984)-74547; polyalkylene oxides as described in Japanese Patent Provisional Publication No. 59(1984)-57231.

The hot-melt solvents preferably are compounds which may be used as solvent of the reducing agent or those which have high dielectric constant and can accelerate physical development of silver salts. Examples of the hot-melt solvents include polyethylene glycols, derivatives of polyethylene oxides (e.g., oleate ester), beeswax, monostearin and high dielectric constant compounds having  $-\text{SO}_2-$  and/or  $-\text{CO}-$  group described in U.S. Pat. No. 3,347,675; polar compounds described in U.S. Pat. No. 3,667,959; and 1,10-decanediol, methyl anisate and biphenyl suberate described in Research Disclosure 26-28 (December 1976). The hot-melt solvent is preferably used in an amount of from 0.5 to 50% by weight, and more preferably from 1 to 20% by weight, based on the total solid content of the light-sensitive layer.

20 The thermal polymerization initiators employable in the light-sensitive material preferably are compounds that are decomposed under heating to generate a polymerization initiating species, particularly a radical, and those commonly employed as initiators of radical polymerization.

25 The thermal polymerization initiators are described in "Addition Polymerization and Ring Opening Polymerization", 6-18, edited by the Editorial Committee of High Polymer Experimental Study of the High Polymer Institute, published by Kyoritsu Shuppan

30 (1983). Examples of the thermal polymerization initiators include azo compounds, e.g., azobisisobutyronitrile, 1,1'-azobis(1-cyclohexanecarbonitrile), dimethyl 2,2'-azobisisobutyrate, 2,2'-azobis(2-methylbutyronitrile), and azobisisdimethylvaleronitrile; organic peroxides, e.g., benzoyl peroxide, di-tert-butyl peroxide, dicumyl peroxide, tert-butyl hydroperoxide, and cumene hydroperoxide; inorganic peroxides, e.g., hydrogen peroxide, potassium persulfate, and ammonium persulfate; and sodium p-toluenesulfonate. The thermal polymerization initiators are preferably used in an amount of from 0.1 to 120% by weight, and more preferably from

35 1 to 10% by weight, based on amount of the polymerizable compound. In a system in which the polymerizable compound located in a portion where the latent image has not been formed is polymerized, the thermal polymerization initiators are preferably incorporated into the light-sensitive layer. The light-sensitive material employing the thermal polymerization initiators is described in Japanese Patent Provisional Publication No. 61(1986)-260241.

40 The development stopping agents employable in the light-sensitive material are compounds that neutralize a base or react with a base to reduce the base concentration in the layer to thereby stop development, or compounds that mutually react with silver or a silver salt to suppress development. More specifically, examples of the development stopping agents include acid precursors capable of releasing acids upon heating electrophilic compounds capable of undergoing substitution

45 reaction with a coexisting base upon heating, nitrogen-containing heterocyclic compounds, mercapto compounds, and the like. Examples of the acid precursors include oxide esters described in Japanese Patent Provisional Publication Nos. 60(1985)-108837 and

50 60(1985)-192939 and compounds which release acids through Lossen rearrangement described in Japanese Patent Provisional Publication No. 60(1985)-230133. Examples of the electrophilic compounds which induce

substitution reaction with bases upon heating are described in Japanese Provisional Publication No. 60(1985)-230134.

The antimudging agents employable in the light-sensitive material preferably are particles which are solid at ambient temperatures. Examples of the antimudging agents include starch particles described in U.K. Pat. No. 1,232,347; polymer particles described in U.S. Pat. No. 3,625,736; microcapsule particles containing no color former described in U.K. Pat. No. 1,235,991; and cellulose particles, and inorganic particles, such as particles of talc, kaolin, bentonite, agalmatolite, zinc oxide, titanium oxide or alumina described in U.S. Pat. No. 2,711,375. Such particles preferably have a mean size of 3 to 50  $\mu\text{m}$ , more preferably 5 to 40  $\mu\text{m}$ . When the microcapsule is employed in the light-sensitive material, the size of said particle is preferably larger than that of the microcapsule.

Examples and usages of the other optional components which can be contained in the light-sensitive layer are also described in the above-mentioned publications and applications concerning the light-sensitive material, and in Research Disclosure Vol. 170, No. 17029, 9-15 (June 1978).

Examples of auxiliary layers which are optionally arranged on the light-sensitive material include an image-receiving layer, a heating layer, an antistatic layer, an anticurl layer and a release layer.

Instead of the use of the image-receiving material, the image-receiving layer can be arranged on the light-sensitive material to produce the desired image on the image-receiving layer of the light-sensitive material. The image-receiving layer of the light-sensitive material can be constructed in the same manner as the material of the image-receiving layer. The details of the image-receiving layer will be described later.

The light-sensitive material employing the heating layer is described in Japanese Patent Application No. 60(1985)-135568 (corresponding to European Patent Provisional Publication No. 203613A). Examples and usage of the other auxiliary layers are also described in the above-mentioned publications and applications concerning the light-sensitive material.

The light-sensitive material of the invention can be prepared, for instance, by the following process.

The light-sensitive material is usually prepared by dissolving, emulsifying or dispersing each of the components of the light-sensitive layer in an adequate medium to obtain coating solution, and then coating the obtained coating solution on a support.

The coating solution can be prepared by mixing liquid compositions each containing a component of the light-sensitive layer. Liquid composition containing two or more components may be also used in the preparation of the coating solution. Some components of the light-sensitive layer can be directly added to the coating solution or the liquid composition. Further, a secondary composition can be prepared by emulsifying the oily (or aqueous) composition in an aqueous (or oily) medium to obtain the coating solution.

The silver halide is preferably prepared in the form of a silver halide emulsion. Various processes for the preparation of the silver halide emulsion are known in the conventional technology for the preparation of photographic materials.

The silver halide emulsion can be prepared by the acid process, neutral process or ammonia process. In the stage for the preparation, a soluble silver salt and a

halogen salt can be reacted in accordance with the single jet process, double jet process or a combination thereof. A reverse mixing method, in which grains are formed in the presence of excess silver ions, or a controlled double jet process, in which a  $\text{pAg}$  value is maintained constant, can also be employed. In order to accelerate grain growth, the concentrations or amounts of the silver salt and halogen salt to be added or the rate of their addition can be increased as described in Japanese Patent Provisional Publication Nos. 55(1980)-142329 and 55(1980)-158124, and U.S. Pat. No. 3,650,757, etc.

The silver halide emulsion may be of a surface latent image type that forms a latent image predominantly on the surface of silver halide grains, or of an inner latent image type that forms a latent image predominantly in the interior of the grains. A direct reversal emulsion comprising an inner latent image type emulsion and a nucleating agent may be employed. The inner latent image type emulsion suitable for this purpose is described in U.S. Pat. Nos. 2,592,250 and 3,761,276, Japanese Patent Publication No. 58(1983)-3534 and Japanese Patent Provisional Publication No. 57(1982)-136641, etc. The nucleating agent that is preferably used in combination with the inner latent image type emulsion is described in U.S. Pat. Nos. 3,227,552, 4,245,037, 4,255,511, 4,266,013 and 4,276,364, and West German Patent Provisional Publication (OLS) No. 2,635,316.

In the preparation of the silver halide emulsions, hydrophilic colloids are advantageously used as protective colloids. Examples of usable hydrophilic colloids include proteins, e.g., gelatin, gelatin derivatives, gelatin grafted with other polymers, albumin, and casein; cellulose derivatives, e.g., hydroxyethyl cellulose, carboxymethyl cellulose, cellulose sulfate, etc.; saccharide derivatives, e.g., sodium alginate and starch derivatives; and a wide variety of synthetic hydrophilic polymers, such as polyvinyl alcohol, polyvinyl alcohol partial acetal, poly-N-vinylpyrrolidone, polyacrylic acid, polymethacrylic acid, polyacrylamide, polyvinylimidazole, and polyvinylpyrazole, and copolymers comprising monomers constituting these homopolymers. Among them, gelatin is most preferred. Examples of employable gelatins include not only lime-processed gelatin, but also acid-processed gelatin and enzyme-processed gelatin. Hydrolysis products or enzymatic decomposition products of gelatin can also be used.

In the formation of silver halide grains in the silver halide emulsion, ammonia, an organic thioether derivative as described in Japanese Patent Publication No. 50 47(1972)-11386 or sulfur-containing compound as described in Japanese Patent Provisional Publication No. 53(1978)-144319 can be used as a silver halide solvent. Further, in the grain formation or physical ripening, a cadmium salt, a zinc salt, a lead salt, a thallium salt, or the like can be introduced into the reaction system. Furthermore, for the purpose of improving high or low intensity reciprocity law failure, a water-soluble iridium salt, e.g., iridium (III) or (IV) chloride, or ammonium hexachloroiridate, or a water-soluble rhodium salt, e.g., rhodium chloride can be used.

After the grain formation or physical ripening, soluble salts may be removed from the resulting emulsion by a known noodle washing method or a sedimentation method. The silver halide emulsion may be used in the primitive condition, but is usually subjected to chemical sensitization. Chemical sensitization can be carried out by the sulfur sensitization, reduction sensitization or noble metal sensitization, or a combination thereof that

are known for emulsions for the preparation of the conventional light-sensitive materials.

When the sensitizing dyes are added to the silver halide emulsion, the sensitizing dye is preferably added during the preparation of the emulsion. When the organic silver salts are introduced in the light-sensitive microcapsule, the emulsion of the organic silver salts can be prepared in the same manner as in the preparation of the silver halide emulsion.

In preparation of the light-sensitive material, the polymerizable compounds are used as the medium for preparation of the liquid composition containing another component of the light-sensitive layer. For example, the silver halide, including the silver halide emulsion), the reducing agent, or the color image forming substance can be dissolved, emulsified or dispersed in the polymerizable compound to prepare the light-sensitive material. Especially, the color image forming substance is preferably incorporated in the polymerizable compound. Further, the necessary components for preparation of microcapsules, such as shell material can be incorporated into the polymerizable compound.

The light-sensitive composition which is the polymerizable compound containing the silver halide can be prepared using the silver halide emulsion. The light-sensitive composition can be also prepared using silver halide powders which can be prepared by lyophilization. These light-sensitive composition can be obtained by stirring the polymerizable compound and the silver halide using a homogenizer, a blender, a mixer or other conventional stirring device.

Polymers having a principal chain consisting essentially of a hydrocarbon chain substituted in part with hydrophilic groups which contain, in their terminal groups, —OH or nitrogen having a lone electron-pair are preferably introduced into the polymerizable compound prior to the preparation of the light-sensitive composition. The polymer has a function of dispersing silver halide or other component in the polymerizable compound very uniformly as well as a function of keeping thus dispersed state. Further, the polymer has another function of gathering silver halide along the interface between the polymerizable compound (i.e., light-sensitive composition) and the aqueous medium in preparation of the microcapsule. Therefore, using this polymer, silver halide can be easily introduced into the shell material of the microcapsule.

The polymerizable compound (including the light-sensitive composition) are preferably emulsified in an aqueous medium to prepare the coating solution. The necessary components for preparation of the microcapsule, such as shell material can be incorporated into the emulsion. Further, other components such as the reducing agent can be added to the emulsion.

The emulsion of the polymerizable compound can be processed for forming the shell of the microcapsule. Examples of the process for the preparation of the microcapsules include a process utilizing coacervation of hydrophilic wall-forming materials as described in U.S. Pat. Nos. 2,800,457 and 2,800,458; an interfacial polymerization process as described in U.S. Pat. No. 3,287,154, U.K. Pat. No. 990,443 and Japanese Patent Publication Nos. 38(1963)-19574, 42(1967)-446 and 42(1967)-771; a process utilizing precipitation of polymers as described in U.S. Pat. Nos. 3,418,250 and 3,660,304; a process of using isocyanate-polyol wall materials as described in U.S. Pat. No. 3,796,669; a process of using isocyanate wall materials as described in

U.S. Pat. No. 3,914,511; a process of using urea-formaldehyde or urea-formaldehyde-resorcinol wall-forming materials as described in U.S. Pat. Nos. 4,001,140, 4,087,376 and 4,089,802; a process of using melamine-formaldehyde resins hydroxypropyl cellulose or like wall-forming materials as described in U.S. Pat. No. 4,025,455; an in situ process utilizing polymerization of monomers as described in U.K. Pat. No. 867,797 and U.S. Pat. No. 4,001,140; an electrolytic dispersion and cooling process as described in U.K. Pat. Nos. 952,807 and 965,074; a spray-drying process as described in U.S. Pat. No. 3,111,407 and U.K. Pat. No. 930,422; and the like. It is preferable, though not limitative, that the microcapsule is prepared by emulsifying core materials containing the polymerizable compound and forming a polymeric membrane (i.e., shell) over the core materials.

The binder is preferably added to the dispersion of the microcapsules to prepare the coating solution of the light-sensitive material. The binder may be dissolved, emulsified or dispersed in the dispersion of the microcapsules. Further, the binder can be dissolved or dispersed in an adequate medium prior to the addition to the dispersion of the microcapsules.

A light-sensitive material of the invention can be prepared by coating and drying the above-prepared coating solution on a support in the conventional manner.

Use of the light-sensitive material is described below.

In the use of the light-sensitive material of the invention, a development process is conducted simultaneously with or after an imagewise exposure.

Various exposure means can be employed in the imagewise exposure, and in general, the latent image on the silver halide is obtained by imagewise exposure to radiation including visible light. The type of light source and exposure can be selected depending on the light-sensitive wavelengths determined by spectral sensitization or sensitivity of silver halide. Original image can be either monochromatic image or color image.

Development of the light-sensitive material can be conducted simultaneously with or after the imagewise exposure. The development can be conducted using a developing solution in the same manner as the image forming method described in Japanese Patent Publication No. 45(1970)-11149. The image forming method described in Japanese Patent Provisional Publication No. 61(1986)-69062 which employs a heat development process has an advantage of simple procedures and short processing time because of the dry process. Thus, the latter method is preferred as the development process of the light-sensitive material.

Heating in the heat development process can be conducted in various known manners. The heating layer which is arranged on the light-sensitive material can be used as the heating means. Heating temperatures for the development process usually ranges from 80° C. to 200° C., and preferably from 100° C. to 160° C. Various heating patterns are applicable. The heating time is usually from 1 second to 5 minutes, and preferably from 5 seconds to 1 minute.

During the above development process, a polymerizable compound in a portion where a latent image of the silver halide has been formed or in a portion where a latent image of the silver halide has not been formed in polymerized. In a general system, the polymerizable compound in a portion where the latent image has been formed is polymerized. If a nature or amount of the

reducing agent is controlled, the polymerizable compound in a portion where the latent image has not been formed can be polymerized in the same manner as the light-sensitive material described in Japanese Patent Provisional Publication No. 61(1986)-260241.

In the above development process, a polymer image can be formed on the light-sensitive layer. A pigment image can be also obtained by fixing pigments to the polymer image.

The image can be also formed on the image-receiving material. The image-receiving material is described hereinbelow. The image forming method employing the image-receiving material or the image-receiving layer is described in Japanese Patent Provisional Publication No. 61(1986)-278849.

Examples of the material employable as the support of the image-receiving material include baryta paper in addition to various examples which can be employed as the support of the known light-sensitive material.

The image-receiving material is usually prepared by providing the image-receiving layer on the support. The image-receiving layer can be constructed according to the color formation system. In the cases that a polymer image is formed on the image-receiving material and that a dye or pigment is employed as the color image forming substance, the image-receiving material may be composed of a simple support.

For example, when a color formation system using a color former and developer is employed, the developer can be contained in the image-receiving layer. Further, the image-receiving layer can be composed of at least one layer containing a mordant. The mordant can be selected from the compounds known in the art of the conventional photography according to the kind of the color image forming substance. If desired, the image-receiving layer can be composed of two or more layers containing two or more mordants different in the mordanting power from each other.

The image-receiving layer preferably contains a polymer as binder. The binder which may be employed in the above-mentioned light sensitive layer is also employable in the image-receiving layer.

The image-receiving layer can be composed of two or more layers according to the above-mentioned functions. The thickness of the image-receiving layer preferably ranges from 1 to 100  $\mu\text{m}$ , more preferably from 1 to 20  $\mu\text{m}$ .

After the development process, pressing the light-sensitive material in contact with the image-receiving material to transfer the polymerizable compounds which is still polymerizable to the image-receiving material, a polymer image can be obtained in the image-receiving material. The process for pressing can be carried out in various known manners.

In the case that the light-sensitive layer contains a color image forming substance, the color image forming substance is fixed by polymerization of the polymerizable compound. Then, pressing the light-sensitive material in contact with the image-receiving material to transfer the color image forming substance in unfixed portion, a color image can be produced on the image-receiving material.

The light-sensitive material can be used for monochromatic or color photography, printing, radiography, diagnosis (e.g., photography for CRT of diagnostic device using supersonic wave), copy (e.g., computer-graphic hard copy), etc.

The present invention is further described by the following examples without limiting the invention.

#### EXAMPLE 1

##### Preparation of silver halide emulsion

In 1,000 ml of water were dissolved 20 g of gelatin and 3 g of sodium chloride, and the resulting gelatin solution was kept at 75°C. To the gelatin solution, 600 ml of an aqueous solution containing 21 g of sodium chloride and 56 g of potassium bromide and 600 ml of an aqueous solution containing 0.59 mole of silver nitrate were added simultaneously at the same feed rate over a period of 40 minutes to obtain a silver chlorobromide emulsion having cubic grains, uniform grain size distribution, mean grain size of 0.35  $\mu\text{m}$  and bromide content of 80 mole %.

The emulsion was washed for desalting and then subjected to chemical sensitization with 5 mg of sodium thiosulfate and 20 mg of 4-hydroxy-6-methyl-1,3,3a,7-tetraazaindene at 60°C. The yield of the emulsion was 600 g.

##### Preparation of light-sensitive composition

In 100 g of trimethylolpropane triacrylate were dissolved 0.40 g of the following copolymer, 6.00 g of Pargascript Red I-6-B (tradename, Ciba-Geigy) and 2 g of Emulex NP-8 (tradename, produced by Nippon Emulsion Co., Ltd.).



To 18.0 g of the resulting solution was dissolved 0.002 g of the following thiol derivative.



To the resulting solution was added a solution in which 0.16 g of the following reducing agent (I) and 1.22 g of the following reducing agent (II) were dissolved in 1.80 g of methylene chloride.





To the solution was further added 3.50 g of the silver halide emulsion, and the resulting mixture was stirred at 15,000 r.p.m. for 5 minutes to obtain a light-sensitive composition. 10

#### Preparation of light-sensitive microcapsule

To 10.51 g of 18.6% aqueous solution of Isobam (tradename, produced by Kuraray Co., Ltd.) was added 48.56 g of 2.89% aqueous solution of pectin. After the solution was adjusted to a pH of 4.0 using 10% sulfuric acid, the light-sensitive composition was added to the resulting solution, and the mixture was stirred at 7,000 r.p.m. for 2 min. to emulsify the light-sensitive composition in the aqueous medium. 15

To 72.5 g of the aqueous emulsion were added 8.32 g of 40% aqueous solution of urea, 2.82 g of 11.3% aqueous solution of resorcinol, 8.56 g of 37% aqueous solution of formaldehyde, and 2.74 g of 8.76% aqueous solution of ammonium sulfate in this order, and the mixture was heated at 60° C. for 2 hours while stirring. After the mixture was adjusted to a pH of 7.0 using 10% aqueous solution of sodium hydroxide, 3.62 g of 30.9% aqueous solution of sodium hydrogen sulfite was added to the mixture to obtain a dispersion containing light-sensitive microcapsules. 25

#### Preparation of light-sensitive material

To 10.0 g of the light-sensitive microcapsule dispersion were added 2 g of 30% aqueous solution of polyvinyl alcohol which has a transmission coefficient of oxygen of  $0.89 \times 10^{-12} \text{ cm}^3 \cdot \text{cm} / \text{cm}^2 \cdot \text{sec} \cdot \text{cmHg}$  at 25° C. (tradename "PVA-205" produced by Kuraray Co., Ltd.) and 1.0 g of 10% solution (solvent: water/ethanol=50/50 as volume ratio) of guanidine trichloroacetate to prepare a coating solution. The coating solution was uniformly coated on a polyethylene terephthalate film (thickness: 100  $\mu\text{m}$ ) using a coating rod of #40 to have a wet thickness of 70  $\mu\text{m}$  and dried at about 40° C. to obtain a light-sensitive material. 35

### EXAMPLE 2

#### Preparation of light-sensitive material

A light-sensitive material was prepared in the same manner as in Example 1 except that 3 g of 30% aqueous solution of gelatin was used in place of 2 g of 30% aqueous solution of polyvinyl alcohol. 40

### COMPARISON EXAMPLE 1

#### Preparation of light-sensitive material

A light-sensitive material was prepared in the same manner as in Example 1 except that 3 g of water was used in place of 2 g of 30% aqueous solution of polyvinyl alcohol. 45

#### Preparation of image-receiving material

To 125 l g of water was added 11 g of 40% aqueous solution of sodium hexametaphosphate, and were further added 34 g of zinc 3,5-di- $\alpha$ -methylbenzylsalicylate and 82 g of 55% aqueous slurry of calcium carbonate, followed by coarsely dispersing in a mixer. The coarse 65

dispersion was then finely dispersed in Dynomill dispersing device. To 200 g of the resulting dispersion were added 6 g of 50% latex of SBR (styrene-butadiene rubber) and 55 g of 8% aqueous solution of polyvinyl alcohol, and the resulting mixture was made uniform. 5

The mixture was then uniformly coated on an art paper having basis weight of 43 g/m<sup>2</sup> to give a layer having a wet thickness of 30  $\mu\text{m}$  dried to obtain an image-receiving material. 10

#### Evaluation of light-sensitive material

Each of the light-sensitive materials prepared in Examples 1 & 2 and Comparison Example 1 was image-wise exposed to light using a tungsten lamp at 2,000 lux for 1 second and then heated on a hot plate at 125° C. for 40 seconds. The exposed and heated light-sensitive material was then combined with the image-receiving material and passed through press rolls under pressure of 350 kg/cm<sup>2</sup> to obtain a magenta positive image on the image receiving material. 20

It was apparent from the results in the inspection of each of the obtained images that the unevenness of the density within the area having a medium density (reflection density of 0.4 to 0.8) was outstanding in the image formed by the light-sensitive material of Comparison Example 1, compared with those of Examples 1 and 2. 25

Further, the condition of dispersion of the microcapsules in the light-sensitive layer was observed using an optical microscope. It was also apparent from the result in the observation that the microcapsules in the light-sensitive material of Comparison Example 1 were remarkably agglutinated. On the other hand, the microcapsules in the materials of Examples 1 and 2 were in the uniformly dispersed state. 30

I claim:

1. In a light-sensitive material comprising a light-sensitive layer which contains silver halide, a reducing agent and a polymerizable compound containing carbon to carbon unsaturation provided on a support, the improvement wherein the silver halide and the polymerizable compound are contained in microcapsules which are dispersed in the light-sensitive layer, and the light-sensitive layer further contains a binder which is arranged outside of the microcapsules. 45
2. The light-sensitive material as claimed in claim 1, wherein the silver halide, the polymerizable compound and the reducing agent are contained in microcapsules in the light-sensitive layer. 50
3. The light-sensitive material as claimed in claim 1, wherein the microcapsules are fixed on the support by the binder. 55
4. The light-sensitive material as claimed in claim 1, wherein the whole surface of the microcapsules is essentially covered with the binder. 60
5. The light-sensitive material as claimed in claim 1, wherein the microcapsules have a mean particle size in the range of from 0.5 to 50  $\mu\text{m}$ . 65
6. The light-sensitive material as claimed in claim 1, wherein the binder is a high molecular weight compound having a molecular weight in the range of from 1,000 to 10,000,000. 70
7. The light-sensitive material as claimed in claim 1, wherein the binder is a polymer having a transmission coefficient of oxygen of not more than  $1.0 \times 10^{-11} \text{ cm}^3 \cdot \text{cm} / \text{cm}^2 \cdot \text{sec} \cdot \text{cmHg}$ . 75
8. The light-sensitive material as claimed in claim 1, wherein the binder in the light-sensitive layer is con- 80

19

tained in an amount of from 10 to 50 weight % based on the amount of the microcapsules.

9. The light-sensitive material as claimed in claim 1, wherein the light-sensitive layer further contains a color image forming substance.

10. In a process for the preparation of a light-sensitive material comprising a light-sensitive layer which contains silver halide, a reducing agent and a polymerizable compound provided on a support, the improvement which comprises:

adding a binder to a microcapsule dispersion containing silver halide, a reducing agent and a polymerizable compound containing carbon to carbon unsaturation to obtain a coating solution, wherein the silver halide and the polymerizable compound are contained in the microcapsules; and

20

coating the coating solution on the support.

11. The process for the preparation of a light-sensitive material as claimed in claim 10, wherein the binder is used in an amount of from 10 to 50 weight % based on the amount of the microcapsules.

12. The light-sensitive material as claimed in claim 1, wherein the binder is a water-insoluble synthetic polymer binder having a transmission coefficient for oxygen of not more than  $1.0 \times 10^{-11} \text{ cm}^3 \cdot \text{cm}/\text{cm}^2 \cdot \text{sec} \cdot \text{cmHg}$ .

10 13. The light-sensitive material as claimed in claim 1, wherein the binder is a polymer selected from the group consisting of polyacrylonitrile, acrylonitrile/styrene copolymer, polymethacrylonitrile, methacrylonitrile/styrene copolymer, polyvinyl chloride, polyvinylidene chloride and vinylidene chloride/acrylonitrile copolymer.

\* \* \* \* \*

20

25

30

35

40

45

50

55

60

65